

# UNITED STATES PATENT OFFICE.

DANIEL TODD MAIN, OF WINNIPEG, MANITOBA, CANADA.

## PROCESS OF CASTING STEEL.

1,327,398.

Specification of Letters Patent. Patented Jan. 6, 1920.

No Drawing.

Application filed June 17, 1918. Serial No. 240,395.

To all whom it may concern:

Be it known that I, DANIEL TODD MAIN, of the city of Winnipeg, in the Province of Manitoba, Canada, have invented certain new and useful Improvements in Processes of Casting Steel, of which the following is the specification.

The invention relates to improvements in processes of casting steel, particularly high speed steel, and the object of the invention is to provide a process which will permit of the direct casting into the shape required of high speed steel and without necessitating forging as is customarily done.

15 The mode of practising my invention is as follows:—

A quantity of high speed steel, such as broken tools usually found in a shop, are put into a crucible and the crucible is heated 20 in a furnace to a high temperature until the steel is melted. After melting, a quantity of manganese and a quantity of silicon are added to the molten mass, the quantity being preferably one per cent. of manganese and 25 one-half per cent. of silicon in proportion to the total weight of the mass in the crucible.

The adding of these materials causes a disturbance in the crucible and the heating is continued until this disturbance subsides. 30 The molten metal is then poured directly into sand molds which have been previously prepared and are of the size and shape of the finished casting which it is desired to produce. The molds and contents are then 35 put back into the furnace and the fire is let die out.

This allows for the gradual cooling of the castings. After an interval of time, that is to say, after the castings have cooled the 40 molds are opened and the castings are removed. They are then cleaned and afterward annealed in the ordinary way in an annealing furnace.

45 After annealing the castings are machined or ground to a finish.

In the above process it is particularly noted that no forging is done, the high speed steel being cast directly into the shape required which may be regular or irregular.

This process is particularly valuable for 50 producing drills and such irregular shaped high speed tools as the tools can be cast directly in the molds into the special shape required and it is only a matter of cleaning and annealing and finally finishing, thereby 55 avoiding having either to forge or machine to shape as is customarily done and allowing of the tremendous saving effected by utilizing broken tools to re-cast new ones.

The finished tool cast by my process is 60 entirely free of blow holes and will maintain a keen cutting edge.

What I claim as my invention is:—

1. The process of casting high speed tools from broken pieces of high speed steel which 65 consists in melting the pieces of steel in a crucible, adding one per cent. of manganese and one-half per cent. of silicon to the molten mass and afterward casting the molten mass in molds previously prepared and 70 of the shape required for the finished tool.

2. The process of casting high speed tools from broken pieces of high speed steel which 75 consists in melting the pieces of steel in a crucible, adding one per cent. of manganese and one-half per cent. of silicon to the molten mass and continuing to heat the mass for a period of time, then pouring the mass directly into previously prepared sand molds of the shape of the tool required and finally 80 cleaning, annealing and machining the casting after the same has cooled.

Signed at Winnipeg, this 28 day of May, 1918.

DANIEL TODD MAIN.

In the presence of—

G. S. ROXBRAUGH,  
K. B. WAKEFIELD.